

## 1

3,028,236

## COLUMBIUM BASE ALLOY

Stanley T. Wlodek, Niagara Falls, Edward D. Weisert, Tonawanda, and Peter M. Moanfeldt, Niagara Falls, N.Y., assignors to Union Carbide Corporation, a corporation of New York  
No Drawing. Filed Dec. 22, 1958, Ser. No. 781,836  
9 Claims. (Cl. 75—174)

This invention relates to a columbium base alloy containing aluminum and vanadium as the major alloying ingredients.

The development of rockets and missiles and advances in nuclear reactors and gas turbines necessitate the use of materials of construction capable of withstanding extreme operating conditions. It is necessary under these conditions to have superior alloys which combine workability, high-temperature strength and high-temperature oxidation resistance.

Accordingly, it is an object of the present invention to provide an alloy which is characterized by resistance to high-temperature oxidation at temperatures in excess of 1000° C.

It is another object of the present invention to provide an alloy which is amenable to heat treatment by conventional means.

Still another object of the present invention is to provide an alloy which, when subjected to an oxidizing atmosphere at elevated temperatures, forms a pellicular metal oxide which adheres firmly to the alloy and is not substantially volatilized therefrom.

Other objects will be apparent from the subsequent disclosure and appended claims.

The alloy which satisfies the objects of the present invention consists essentially of 0.5 to 10 weight percent aluminum, 0.5 to 10 weight percent vanadium, up to 40 weight percent titanium, up to 30 weight percent chromium, up to 30 weight percent in the aggregate of at least one metal selected from the group consisting of tungsten and tantalum, up to 10 weight percent in the aggregate of at least one metal selected from the group consisting of manganese, nickel, iron, cobalt, zirconium and hafnium, up to 5 weight percent in the aggregate of at least one alloying element selected from the group consisting of barium, silicon, beryllium, yttrium, boron and the rare earth metals, and the remainder being columbium in a minimum amount of at least 30 weight percent.

In the foregoing alloys, the columbium content is advantageously in excess of 45 percent and preferably in excess of 70 percent.

Even where the alloy has a very high columbium content, the addition thereto of small amounts of the aluminum and vanadium greatly enhances the alloy's properties. For example, an alloy containing about 4 weight percent each of aluminum and vanadium, the balance being columbium and incidental impurities exhibits superior properties. If, in addition to the aluminum and vanadium, about 7 weight percent of titanium is added, the properties of the alloy are still further enhanced.

While the foregoing alloy satisfies all of the objects set forth above it has been found that an alloy consisting essentially of 1 to 25 weight percent titanium, 1 to 15 weight percent chromium, 1 to 6 weight percent aluminum, 0.5 to 6 weight percent vanadium, up to 30 weight percent in the aggregate of at least one metal selected from the group consisting of tungsten and tantalum, up to 5 weight percent in the aggregate of at least one metal selected from the group consisting of manganese, nickel, iron, cobalt, zirconium and hafnium, up to 3 weight percent in the aggregate of at least one alloying element selected from the group consisting of barium, silicon, beryllium, yttrium, boron and the rare earth metals, and

## 2

the remainder being columbium in a minimum amount of at least 45 weight percent is particularly outstanding for use under oxidizing conditions and particularly high-temperature oxidizing conditions since the alloy strongly resists reaction with oxygen at temperatures in excess of 1100° C.

The maximum benefits of the present alloy are obtained when the alloy consists essentially of from 5 to 20 weight percent titanium, 3 to 12 weight percent chromium, 2 to 6 weight percent aluminum, 1 to 5 weight percent vanadium, up to 30 weight percent in the aggregate of at least one metal selected from the group consisting of tungsten and tantalum, up to 5 weight percent in the aggregate of at least one metal selected from the group consisting of manganese, nickel, iron, cobalt, zirconium, and hafnium, up to 3 weight percent in the aggregate of at least one alloying element selected from the group consisting of barium, silicon, beryllium, yttrium, boron and the rare earth metals, and the remainder being columbium in a minimum amount of at least 50 weight percent.

Within the compositional ranges set forth above, certain specific compositions have been found to have exceptional properties. These compositions are shown in Table I which follows:

TABLE I  
Alloy Composition

| Percent: | 63 | 75 | 59 | 72 |
|----------|----|----|----|----|
| Cb       | 20 | 10 | 20 | 10 |
| Ti       | 9  | 8  | 9  | 9  |
| Cr       | 5  | 4  | 5  | 4  |
| V        | 3  | 3  | 3  | 3  |
| Al       |    |    | 4  | 2  |
| Fe       |    |    |    |    |

The alloys of the present invention may be prepared by any number of methods such as the conventional methods using inert operating conditions, e.g., by the consumable arc-melting technique described in U.S. Patent No. 2,640,860, by non-consumable arc welding, by pressing and sintering of metallic powders or by other powder metallurgical processes. Great caution should be exercised to protect the metals from the atmosphere since contamination of the alloying mass by nitrogen and oxygen, etc. destroys many of the valuable properties of the alloy.

To protect the alloying materials from these atmospheric contaminants the alloying operation should be performed under vacuum or in an inert atmosphere, such as argon or helium, or under a protective slag or under a combination of protective slag and controlled atmosphere. The final shaping of the alloy metal may be accomplished after cooling by any of several procedures, such as, extrusion, swaging, rolling or grinding the cast or sintered shape.

The examples provided below are prepared in a non-consumable arc furnace such as that described by W. Kroll in Transactions of the Electro-Chemical Society, volume 78, 1940, pages 35 through 47. The procedure consists of placing the component metals on a water cooled, copper crucible shaped to retain the charge in a hearthlike depression and incorporated in a gas tight container supplied with a tungsten electrode capable of impressing an arc onto the charge. After careful evacuation of the system the charge was melted four times under an argon atmosphere until a homogeneous alloy of the desired composition was obtained.

The oxidation resistance of the alloy was determined by exposing highly polished specimens measuring approximately 1.60 x 0.85 x 0.65 centimeters to a stream of pure, dry oxygen within an air tight container. The specimens were suspended and heated in this atmosphere at 800° C., 1000° C., or 1200° C. and the amount of pellicular metal oxide formed on the surfaces during the exposure was continuously measured and recorded auto-

matically by means of balances of the Mauer type. By this method an accurate rate of oxidation weight gain could be obtained for the alloys tested. The weight gain is expressed in milligrams of weight gained per square centimeter of surface exposed for at least 100 hours at the different temperatures.

#### EXAMPLE I

Adopting the procedures described above, an alloy was prepared containing 57 percent columbium, 20 percent titanium, 5 percent iron, 10 percent chromium, 4 percent aluminum, and 4 percent vanadium. Upon testing for its oxidation resistance, the 100 hour weight gain, expressed in milligrams per square centimeter, was found to be 9.68 at 800° C., 48.1 at 1000° C., and 132.0 at 1200° C. Unalloyed columbium showed weight gains of 3630 milligrams per square centimeter at 800° C., 6670 milligrams per square centimeter at 1000° C., and 24,000 milligrams per square centimeter at 1200° C. under identical testing conditions.

#### EXAMPLE II

Adopting the procedures described above, an alloy was prepared containing 57 percent columbium, 20 percent titanium, 5 percent nickel, 10 percent chromium, 4 percent aluminum, and 4 percent vanadium. Upon testing for its oxidation resistance, the 100 hour weight gain, expressed in milligrams per square centimeter, was found to be 5.85 at 800° C., 32.4 at 1000° C., and 189.4 at 1200° C.

#### EXAMPLE III

Adopting the procedures described above, an alloy was prepared containing 60.2 percent columbium, 18.3 percent titanium, 3.3 percent nickel, 3.3 percent iron, 8.3 percent chromium, 3.3 percent aluminum, and 3.3 percent vanadium. Upon testing for its oxidation resistance, the 100 hour weight gain expressed in milligrams per square centimeter, was found to be 14.7 at 800° C., 30.5 at 1000° C. and 193 at 1200° C.

#### EXAMPLE IV

Adopting the procedures described above, an alloy was prepared containing 63 percent columbium, 20 percent titanium, 9 percent chromium, 5 percent vanadium and 3 percent aluminum. Upon testing for its oxidation resistance, the 100 hour weight gain, expressed in milligrams per square centimeter, was found to be 12.5 at 800° C., 61.6 at 1000° C. and 184 at 1200° C.

#### EXAMPLE V

Adopting the procedures described above, an alloy was prepared containing 63.5 percent columbium, 20 percent titanium, 9 percent chromium, 4 percent vanadium, 3 percent aluminum, and 0.5 percent zirconium. Upon testing for its oxidation resistance, the 100 hour weight gain, expressed in milligrams per square centimeter, was found to be 8.71 at 800° C., 69.7 at 1000° C. and 315 at 1200° C.

#### EXAMPLE VI

Adopting the procedures described above, an alloy was prepared containing 46 percent columbium, 35 percent titanium, 8 percent chromium, 4 percent vanadium, 3 percent aluminum, and 4 percent manganese. Upon testing for its oxidation resistance, the 100 hour weight gain, expressed in milligrams per square centimeter, was found to be 12.5 at 800° C., 134 at 1000° C. and 342 at 1200° C.

#### EXAMPLE VII

Adopting the procedures described above, an alloy was prepared containing 53 percent columbium, 20 percent titanium, 3 percent vanadium, 3 percent aluminum, 3 percent chromium, 3 percent cobalt, 3 percent iron, 3 percent nickel, 3 percent silicon, 3 percent tantalum and 3 percent tungsten. Upon testing for its oxidation resistance, the 100 hour weight gain, expressed in milligrams

per square centimeter was found to be 3.8 at 800° C., 23.8 at 1000° C. and 65.5 at 1200° C.

#### EXAMPLE VIII

Adopting the procedures described above, an alloy was prepared containing 90 percent columbium, 5 percent aluminum and 5 percent vanadium. Upon testing for its oxidation resistance, the 100 hour weight gain, expressed in milligrams per square centimeter, was found to be 98.8 at 1000° C.

#### EXAMPLE IX

Adopting the procedures described above, an alloy was prepared containing 94 percent columbium, 3 percent aluminum and 3 percent vanadium. Upon testing for its oxidation resistance, the 100 hour weight gain, expressed in milligrams per square centimeter, was found to be 46 at 800° C. and 92.2 at 1000° C.

#### EXAMPLE X

Adopting the procedures described above, an alloy was prepared containing 90 percent columbium, 7 percent aluminum and 3 percent vanadium. Upon testing for its oxidation resistance, the 100 hour weight gain, expressed in milligrams per square centimeter, was found to be 18.9 at 800° C. and 140 at 1000° C.

#### EXAMPLE XI

Adopting the procedures described above, an alloy was prepared containing 70 percent columbium, 5 percent aluminum, 5 percent vanadium and 20 percent tantalum. Upon testing for its oxidation resistance, the 100 hour weight gain, expressed in milligrams per square centimeter, was found to be 24.2 at 800° C. and 122 at 1000° C.

#### EXAMPLE XII

Adopting the procedures described above, an alloy was prepared containing 72 percent columbium, 5 percent aluminum, 5 percent vanadium and 20 percent titanium. Upon testing for its oxidation resistance, the 100 hour weight gain, expressed in milligrams per square centimeter, was found to be 13.6 at 800° C. and 105 at 1000° C.

Although it is preferable to use high-purity metals in the preparation of the alloys of the present invention, a small amount of variance in purity can be tolerated before product quality suffers appreciably. The alloys of the working examples are prepared from commercially available metals which contain a small percentage of incidental impurities.

#### What is claimed is:

50. 1. An alloy consisting essentially of from 1 to 25 weight percent titanium, 1 to 15 weight percent chromium, 1 to 6 weight percent aluminum, 0.5 to 6 weight percent vanadium, up to 30 weight percent in the aggregate of at least one metal selected from the group consisting of tungsten and tantalum, up to 5 weight percent in the aggregate of at least one metal selected from the group consisting of manganese, nickel, cobalt, iron, zirconium, and hafnium, up to 3 weight percent in the aggregate of at least one alloying element selected from the group consisting of barium, silicon, beryllium, yttrium, boron and the rare earth metals, the remainder being columbium in a minimum amount of at least 45 weight percent.
55. 2. An alloy consisting essentially of from 5 to 20 weight percent titanium, 3 to 12 weight percent chromium, 2 to 6 weight percent aluminum, 1 to 5 weight percent vanadium, up to 30 weight percent in the aggregate of at least one metal selected from the group consisting of tungsten and tantalum, up to 5 weight percent in the aggregate of at least one metal selected from the group consisting of manganese, nickel, iron, cobalt, zirconium, and hafnium, up to 3 weight percent in the aggregate of at least one alloying element selected from the group consisting of barium, silicon, beryllium, yttrium, boron and the rare earth metals, and the remainder being columbium in a minimum amount of at least 50 weight percent.

3. An alloy consisting essentially of about 20 weight percent titanium, about 9 weight percent chromium, about 5 weight percent vanadium, about 3 weight percent aluminum, the balance being columbium and incidental impurities.

4. An alloy consisting essentially of about 10 weight percent titanium, about 8 weight percent chromium, about 4 weight percent vanadium, about 3 weight percent aluminum, the balance being columbium and incidental impurities.

5. An alloy consisting essentially of about 20 weight percent titanium, about 9 weight percent chromium, about 5 weight percent vanadium, about 4 weight percent iron, about 3 weight percent aluminum, the balance being columbium and incidental impurities.

6. An alloy consisting essentially of about 10 weight percent titanium, about 9 weight percent chromium, about 4 weight percent vanadium, about 3 weight percent aluminum, about 2 weight percent iron, the balance being columbium and incidental impurities.

7. An alloy consisting essentially of about 4 weight percent aluminum, about 4 weight percent vanadium, the balance being columbium and incidental impurities.

8. An alloy consisting essentially of about 7 weight percent titanium, about 4 weight percent aluminum, about 4 weight percent vanadium, the balance being columbium and incidental impurities.

9. An alloy consisting essentially of from .5 to 10 weight percent aluminum, from .5 to 10 weight percent vanadium, the balance being columbium and incidental impurities.

References Cited in the file of this patent

UNITED STATES PATENTS

|    |           |            |               |
|----|-----------|------------|---------------|
| 15 | 2,822,268 | Hix        | Feb. 4, 1958  |
|    | 2,838,395 | Rhodin     | June 10, 1958 |
|    | 2,838,396 | Rhodin     | June 10, 1958 |
|    | 2,860,970 | Thielemann | Nov. 18, 1958 |
| 20 | 2,882,146 | Rhodin     | Apr. 14, 1959 |
|    | 2,883,282 | Wainer     | Apr. 21, 1959 |